

## UNITED STATES PATENT OFFICE

2,412,217

FROTH FLOTATION OF CHROMITE  
WITH FLUORIDE

Richard Havens, Salt Lake City, Utah, assignor to  
the United States of America, as represented by  
the Secretary of the Interior

No Drawing. Application December 19, 1944,  
Serial No. 568,908

5 Claims. (Cl. 209—166)

(Granted under the act of March 3, 1883, as  
amended April 30, 1928; 370 O. G. 757)

1

The invention described herein may be manufactured and used by or for the Government of the United States for governmental purposes without the payment to me of any royalty thereon in accordance with the provisions of the act of April 30, 1928 (Ch. 460, 45 Stat. L. 467).

This invention relates to the beneficiation of chromium ores, and more particularly to the production of a chromite ore concentrate. Heretofore, attempts have been made to beneficiate chromium ores by magnetic separation, gravity concentration, and flotation methods but in the case of gravity or magnetic methods very expensive equipment is required and the flotation methods have not been particularly satisfactory from the standpoint of yields and quantities of reagents employed.

Accordingly, this invention has as an object the provision of a practical and economical process for the beneficiation of chromium ores. Another object is to provide a mineral concentrating treatment for the beneficiation of chromium ores involving selective filming of a desired mineral and the production of a high-grade chromium containing concentrate. A further object is the provision of a flotation process or other mineral filming treatment wherein a high grade of concentrate is produced with maximum recovering of chromium-bearing material with a very low consumption of reagents. Other and further objects will be apparent or will appear hereinafter as this specification proceeds.

These objects are accomplished in accordance with this invention wherein chromium ores are beneficiated by subjecting them to a mineral-concentrating treatment involving selective filming under acidic conditions in the presence of a soluble fluoride. Desirably, a soluble fluorine compound capable of yielding fluoride ions under acidic conditions is employed. While agglomeration tabling concentrating treatments, bulk flotation and similar mineral concentrating treatments involving selective filming of one or more ore constituents can be employed, it is preferred to employ a froth flotation concentration involving agitation and aeration of an aqueous pulp of a comminuted chromium-bearing ore, and the ensuing description will largely be directed to this type of mineral concentrating treatment.

Suitable chromium ores for employment in ac-

2

cordance with this invention include any of the usual ores from which chromium is derived such as for example Oregon beach sands containing chromite, the residues from gravity separation plants formerly discarded, and other similar chromite-containing ores.

Suitable soluble fluorides for employment in accordance with this invention include any fluorine compound which is soluble in an aqueous menstruum or pulp, or which becomes soluble therein under acidic conditions ranging from the strongly acid to the moderately acid pH range. Examples of suitable fluorine compounds are hydrofluoric acid, the alkali metal fluorides such as sodium, potassium and lithium fluoride, the soluble silicofluorites such as sodium and potassium and ammonium silicofluorite, and similar ionizable fluorine compounds which are appreciably soluble in water at a pH range between about pH 1.5 and pH 5.5.

The beneficiation of chromium ores for example chromites, is carried out under acidic conditions ranging from the strongly acid to the moderately acid and generally within a pulp acidity of between pH 1.5 and pH 5.5 preferably, however, the pulp acidity is maintained within the more restricted pH range of between pH 2.5 and pH 4.5 in order that the acidity cooperate to best advantage with the soluble fluoride to accomplish a good recovery of high-grade chromite concentrate. While the exact function of the soluble fluoride in this method for beneficiating chromium ores is not entirely understood, and therefore it is not desired to limit this invention to any particular theory of reaction, nevertheless it is thought that the soluble fluoride under acidic conditions accomplishes several things among which may be mentioned the cleaning of the mineral surface, the dispersion of slimes, the depression of undesired gangue materials such as garnet, ilmenite, quartz and the like, and the selective activation of the chromite particles enabling them to be readily floated away from gangue constituents.

In carrying out the beneficiation of chromium ores, the ores are preferably ground by customary means to provide liberation of the chromite or other chromium-bearing material from the gangue constituents, and generally the chromium-bearing ore is comminuted to particle size between

minus 20-mesh and minus 800-mesh; preferably the particle size of the ore is maintained within the more restricted range of between minus 48-mesh and minus 200-mesh.

By the expression "minus —-mesh" is meant a particle size which passes through a standard Tyler screen having the stated number of meshes per linear inch.

In general, it has been found that superior results are secured when the selected chromium ore is stage ground and when it is deslimed, that is to say freed from particles having diameters less than 10 microns, prior to the treatment of this invention. In desliming the ore, treatment with a small amount of sodium silicate appears to facilitate dispersion of the slimes and their subsequent removal, as by washing of the desired sands with a large excess of water. A suitable amount of sodium or other soluble silicate is from 1 to 10 pounds of soluble silicate per ton of ore.

In the practice of this invention, it has been found that the employment of a long chain fatty acid having from 8 to 18 carbon atoms as a collector or collecting agent results in a superior grade and recovery of chromium concentrate when employed in conjunction with the acidic pulp and the soluble fluoride of this invention. Suitable long chain fatty acids, generally employed in amounts of from 0.5 to 5 pounds per ton of ore and preferably within the more restricted range of from about 1 to 4.5 pounds of fatty acid per ton of ore, include the fatty acids derived from vegetable, animal, marine and synthetic sources having from 8 to 18 carbon atoms in the molecule, examples being the fatty acids derived from olive oil, palm oil, coconut oil, castor oil, sunflower seed oil, sesame oil, linseed oil, whale oil, sardine oil, menhaden oil, and the synthetic fatty acids produced in the oxidation of petroleum and similar hydrocarbons. Lauric acid, palmitic acid, stearic acid and preferably oleic acid have been found eminently suitable for employment in this invention.

Highly efficient results and considerable reagent economy have been effected in the practice of this invention when the fatty acid collector employed is incorporated in the form of a stabilized emulsion or dispersion with the ore pulp, and to this end it is preferred to employ a small amount of a dispersing agent together with the fatty acid, a suitable dispersing agent being the ammonium salt of lauryl diethylene glycol sulfate sold by the Emulsol Corporation of Chicago, Illinois, under the trade name "Emulsol X-1." Other dispersing agents stable to acidic conditions can, of course, be employed to achieve the same and, representative examples being starch, salts of long chain amines, and alkylol amine salts of the fatty acids themselves. "Emulsol X-1" as above defined however constitutes a preferred dispersing agent for use. The dispersing agent, generally employed in amounts of from .1 to 2.5 pounds per ton of ore and preferably in an amount within the more restricted ores from 0.2 to 2.0 pounds per ton of ore, is preferably incorporated with a suitable amount of water and with the selected long chain fatty acid such as oleic acid prior to its incorporation with the ore pulp for greatest reagent economy.

To achieve the desirable acidic pulp conditions in accordance with this invention, one may employ hydrofluoric acid itself to supply both the soluble fluoride and the necessary pH range as above discussed, but in general it has been found equally satisfactory to employ other strong min-

eral acids, generally in amounts of from 1 to 11 pounds of acid per ton of ore, and preferably from about 3 to about 7 pounds of acid per ton of ore, such as for example nitric acid, hydrochloric acid, and preferably the cheap and readily available sulfuric acid. Sulfuric acid has the additional advantage in this invention of removing soluble calcium salts from the pulp and thereby preventing any interference with the mineral concentrating treatment which might result from the presence of soluble calcium salts in the pulp.

In carrying out this invention in accordance with the foregoing principles, the selected chromium ore is ground in a suitable device such as a ball mill, then preferably although not necessarily deslimed by washing with an excess of water to remove colloidally dispersed material, and thereafter the sands are diluted to a pulp consistency of generally about 25 percent solids. Thereafter, the pulp is conditioned by agitating with an amount of strong mineral acid sufficient to bring the pH range of the pulp within the desired acidity, and the fatty acid collector (preferably emulsified or dispersed with the dispersing agent selected), is incorporated with the pulp. Thereafter, the soluble fluoride is incorporated in the selected amount, the pulp is conditioned for a suitable length of time, and flotation is initiated. Any suitable flotation machine can be employed, such as for example the Denver Cell or the Callow type of flotation machine. The usual rougher and cleaner procedures are employed and this invention can well be utilized in a cyclic process wherein in the tailing water and middling ore fractions are returned to the process.

The following illustrative examples show how the invention may be carried out, but it is not limited thereto. Parts and percentage compositions are by weight unless otherwise designated.

#### EXAMPLE I

##### ORE: MOUAT CHROMITE

*Treatment.*—This sample represents consolidated ores requiring grinding for liberation of the chromite from which chromite may be recovered by flotation. Ore roll crushed minus 10-mesh was stage ground minus 48-mesh and deslimed. Sands were conditioned ½-hour with  $H_2SO_4$  solution and deslimed. Sands were pulped, conditioned and chromite floated. Chromite concentrate cleaned and recleaned.

Table 1  
REAGENTS, POUNDS PER TON OF ORE

| 55 |  | Cond.     | Rougher | Cleaner    | Recleaner     |
|----|--|-----------|---------|------------|---------------|
|    |  | $H_2SO_4$ | NaF     | Oleic acid | "Emulsol X-1" |
|    |  | 5.8       | 3.33    | 1.66       | 1.66          |
|    |  |           | 3.33    | 1.66       | 1.66          |
|    |  |           | 1.33    | .50        | .25           |
|    |  |           |         | .27        | .10           |
| 60 |  |           |         |            | .05           |

##### METALLURGICAL DATA

| 65 | Product           | Per cent wt. | Assay, per cent |      |         | Distribution, per cent |       |
|----|-------------------|--------------|-----------------|------|---------|------------------------|-------|
|    |                   |              | $Cr_2O_3$       | Fe   | $SiO_2$ | $Cr_2O_3$              | Fe    |
|    | Chromite conc. 1. | 37.9         | 41.4            | 22.0 | 1.8     | 62.2                   | 50.3  |
|    | Chromite conc. 2. | 9.5          | 39.4            | 20.8 | 5.2     | 14.8                   | 11.9  |
|    | Recleaner tailing | 4.3          | 22.3            | 17.2 | —       | 3.9                    | 4.5   |
|    | Cleaner tailing   | 9.3          | 16.3            | 14.6 | —       | 6.0                    | 8.2   |
|    | Rougher tailing   | 31.0         | 7.0             | 9.9  | —       | 8.6                    | 18.5  |
|    | Slimes            | 8.0          | 14.0            | 13.8 | —       | 4.5                    | 6.6   |
|    | Calculated heads  | 100.0        | 25.2            | 16.6 | —       | 100.0                  | 100.0 |
| 70 | Combined concs    | 47.4         | 41.0            | 21.8 | 2.5     | 77.0                   | 62.2  |

**5**  
**EXAMPLE II**

**ORE: CASTRO CHROMITE SLIMES**

*Treatment.*—This sample represents a source of chromite losses as tailing from a typical flotation mill from which chromite can be recovered by flotation to improve plant metallurgy. A sample of slimes as received was pulped with sodium silicate and deslimed. Sands were pulped, conditioned, and chromite floated. Chromite concentrates were cleaned and recleaned.

**Table 2**  
**REAGENTS, POUNDS PER TON OF ORE**

|                                      | Desliming | Rougher | Cleaner | Recleaner |
|--------------------------------------|-----------|---------|---------|-----------|
| Sodium silicate.....                 | 26.2      | 3.7     |         | 1.8       |
| NaF.....                             |           | 4.6     | 0.9     | .9        |
| Oleic acid.....                      |           | .9      | 1       | 1         |
| H <sub>2</sub> SO <sub>4</sub> ..... |           | 5.8     | 2.5     | 1.8       |
| "Emulsol X-1".....                   |           | .2      | .02     | .02       |

**METALLURGICAL DATA**

| Product                | Wt., per cent | Assay, per cent                |      | Distribution, per cent         |       |
|------------------------|---------------|--------------------------------|------|--------------------------------|-------|
|                        |               | Cr <sub>2</sub> O <sub>3</sub> | Fe   | Cr <sub>2</sub> O <sub>3</sub> | Fe    |
|                        |               | 9.33                           | 40.8 | 11.85                          | 37.3  |
| Chromite conc. 1.....  |               | 2.19                           | 34.1 | 10.25                          | 3.7   |
| Chromite conc. 2.....  |               | 3.84                           | 19.3 | 7.2                            | 4.7   |
| Recleaner tail. 2..... |               | 11.33                          | 18.1 | 7.2                            | 20.0  |
| Recleaner tail. 1..... |               | 7.31                           | 11.4 | 6.0                            | 8.1   |
| Cleaner tail.....      |               | 39.86                          | 1.8  | 4.1                            | 7.1   |
| Rougher tail.....      |               | 26.14                          | 5.1  | 5.6                            | 13.0  |
| Calculated heads.....  | 100.00        | 10.2                           | 6.0  | 100.0                          | 100.0 |
| Combined concs.....    | 11.52         | 39.6                           | 11.5 | 44.6                           | 22.3  |

*Remarks.*—Slimes as received contained 73.0 percent minus 200-mesh and sands floated contained 73.5 percent minus 200-mesh.

5  
The unconsolidated sands as received were screen sized and results are given in Table 3.

**6**  
**EXAMPLE III**

**SCREEN ANALYSES**

**Table 3**  
**SCREEN ANALYSIS OF HUMPHREYS GOLD CORPORATION CONCENTRATES**

| Product               | Wt., per cent | Assay, per cent                |      | Distribution, per cent         |        |
|-----------------------|---------------|--------------------------------|------|--------------------------------|--------|
|                       |               | Cr <sub>2</sub> O <sub>3</sub> | Fe   | Cr <sub>2</sub> O <sub>3</sub> | Fe     |
| +48-mesh.....         |               | 4.35                           | 10.3 | 23.3                           | 2.00   |
| -48+100-mesh.....     |               | 37.46                          | 22.6 | 88.15                          | 92.41  |
| -100+200-mesh.....    |               | 8.19                           | 27.0 | 23.9                           | 9.85   |
| Calculated heads..... | 100.00        | 22.5                           | 28.0 | 100.00                         | 100.00 |

**CHEMICAL ANALYSES, PER CENT**

|                      | Cr <sub>2</sub> O <sub>3</sub> | Fe   | SiO <sub>2</sub> | MgO | Al <sub>2</sub> O <sub>3</sub> | CaO | ZrO <sub>2</sub> | TiO <sub>2</sub> |
|----------------------|--------------------------------|------|------------------|-----|--------------------------------|-----|------------------|------------------|
| Humphreys Gold Corp. | 24.60                          | 21.0 | 15.9             | 4.2 | 17.4                           | 1.0 | -----            | -----            |

30  
35  
30  
35  
40  
Beach sands as received were pulped with Salt Lake City tap water to about 50 percent solids and an emulsion of oleic acid stabilized with "Emulsol X-1" was added until flocculation was fairly complete. Sodium fluoride was added in stages until some depression of the garnet was noted. The pulp was then diluted to about 25 percent solids and dilute sulfuric acid was added until flocs were clean of garnet and gangue. The flocculated chromite then floated rapidly and usually no additional collector was required.

Results of flotation tests on Humphreys Gold Corporation primary concentrates are given in Tables 4, 5, and 6, except that magnetic separation was employed on the chromite cleaner concentrates in the test recorded in Table 4.

**Table 4**  
**CHROMITE FLOTATION USING LARGE AMOUNTS OF FATTY ACID**

| Product                                              | Wt., percent | Assay, percent                 |      |                  | Distribution, percent          |       |                  | Ratio Cr/Fe |
|------------------------------------------------------|--------------|--------------------------------|------|------------------|--------------------------------|-------|------------------|-------------|
|                                                      |              | Cr <sub>2</sub> O <sub>3</sub> | Fe   | SiO <sub>2</sub> | Cr <sub>2</sub> O <sub>3</sub> | Fe    | SiO <sub>2</sub> |             |
| Chromite cleaner concentrate 1.....                  | 49.4         | 43.10                          | 21.0 | 1.0              | 84.4                           | 54.9  | 2.9              | 1.40        |
| Chromite cleaner concentrate 2.....                  | 3.1          | 35.32                          | 21.0 | 3.6              | 4.3                            | 3.4   | 0.6              | 1.15        |
| Chromite cleaner tailing.....                        | 11.4         | 23.80                          | 22.0 | 9.0              | 10.8                           | 13.3  | 6.0              | 0.78        |
| Rougher tailing.....                                 | 36.1         | 0.32                           | 14.8 | 42.8             | 0.5                            | 28.4  | 90.5             | -----       |
| Calculated head.....                                 | 100.0        | 25.19                          | 18.9 | 17.1             | 100.0                          | 100.0 | 100.0            | -----       |
| Nonmagnetic from chromite cleaner concentrate 1..... | 44.0         | 46.7                           | 19.8 | 0.8              | 79.8                           | 45.2  | 2.6              | 1.62        |
| Magnetic from chromite cleaner concentrate 1.....    | 5.4          | 22.0                           | 34.1 | 0.6              | 4.6                            | 9.7   | 0.3              | -----       |
| Calculated head chromite cleaner concentrate.....    | 49.4         | 43.8                           | 21.4 | 0.8              | 84.4                           | 54.9  | 2.9              | -----       |

**REAGENTS, POUNDS PER TON OF ORE**

|                        | Oleic acid | "Emulsol X-1" | NaF  | H <sub>2</sub> SO <sub>4</sub> | pH  |
|------------------------|------------|---------------|------|--------------------------------|-----|
| Rougher flotation..... |            | 4.12          | 0.82 | 11.8                           | 2.7 |
| Cleaner flotation..... |            | 1.75          | 0.35 | 4.7                            | 5.9 |

The results recorded in Table 4 show that 99.5 percent of the chromium was recovered in a rougher concentrate that assayed 39.3 percent Cr<sub>2</sub>O<sub>3</sub>. Final cleaner flotation concentrate showed a recovery of 88.4 percent of the chromium, assayed 43.1 per cent Cr<sub>2</sub>O<sub>3</sub>, 21 percent iron, 1.0 percent SiO<sub>2</sub>, and had a chromium to iron ratio of 1.40.

By using low intensity magnetic separation to reject magnetite and ilmenite from the chromite cleaner concentrate, 79.8 percent of the total chromium was recovered in a nonmagnetic product that assayed 46.7 percent Cr<sub>2</sub>O<sub>3</sub>, 19.8 percent Fe, 0.8 percent SiO<sub>2</sub> and had a chromium to iron ratio of 1.62 to 1.

By flotation, 95.0 percent of the chromium was recovered in a rougher concentrate that assayed 38.8 percent Cr<sub>2</sub>O<sub>3</sub>. The final chromite cleaner concentrate represented an 84.2 percent recovery of the chromium and assayed 41.50 percent Cr<sub>2</sub>O<sub>3</sub>, 23.0 percent Fe and 1.0 percent SiO<sub>2</sub>. Results were comparable to those given in Table 5 and reagent consumption was lower.

#### EXAMPLE IV

##### PIONEER MINE SANDS

The following flotation tests recorded in Tables 7, 8, 9, and 10 were made on sands from the Pioneer mine. Procedure for flotation on these sands 15 differs somewhat from procedure used in the flo-

Table 5

| Product                        | Wt., percent | Assay, percent                 |      |                  | Distribution, percent          |       |                  | Ratio Cr/Fe |
|--------------------------------|--------------|--------------------------------|------|------------------|--------------------------------|-------|------------------|-------------|
|                                |              | Cr <sub>2</sub> O <sub>3</sub> | Fe   | SiO <sub>2</sub> | Cr <sub>2</sub> O <sub>3</sub> | Fe    | SiO <sub>2</sub> |             |
| Chromite cleaner concentrate 1 | 46.6         | 42.00                          | 20.8 | 1.0              | 80.6                           | 44.9  | 3.1              | 1.38        |
| Chromite cleaner concentrate 2 | 4.5          | 33.72                          | 28.4 | 1.6              | 6.2                            | 5.8   | 0.5              | .79         |
| Chromite cleaner tailing       | 8.8          | 21.35                          | 25.8 | 9.0              | 7.7                            | 10.5  | 5.2              | -----       |
| Rougher tailing                | 40.1         | 3.33                           | 20.9 | 34.3             | 5.5                            | 38.8  | 91.2             | -----       |
| Calculated heads               | 100.0        | 24.32                          | 21.6 | 15.0             | 100.0                          | 100.0 | 100.0            | -----       |

## REAGENTS, POUNDS PER TON OF ORE

|                   | Oleic acid | "Emulsol X-1" | NaF  | H <sub>2</sub> SO <sub>4</sub> | pH    |
|-------------------|------------|---------------|------|--------------------------------|-------|
| Rougher flotation | 1.49       | 0.30          | 2.98 | 2.19                           | 3.8   |
| Cleaner flotation | .25        | 0.05          | 2.39 | 1.00                           | ----- |

The results given in Table 4 show a recovery of 94.5 percent of the chromium in a rougher concentrate that assayed 38.4 percent Cr<sub>2</sub>O<sub>3</sub>. However, 80.6 percent of the chromium was recovered in the final chromite cleaner concentrate that contained 42.00 percent Cr<sub>2</sub>O<sub>3</sub>, 20.8 percent Fe and 1.0 percent SiO<sub>2</sub>. Smaller amounts of reagents were used in this test than in the one recorded in Table 4, but recovery of chromium was not quite as good.

tation of chromite from Humphreys Gold Corporation sands. The major object was to verify substitution of hydrofluoric acid for the fluoridesulfuric acid circuit and study the effect of de-40 pressant addition ahead of fatty acid.

## CHEMICAL ANALYSES, PER CENT

|                 | Cr <sub>2</sub> O <sub>3</sub> | Fe   | SiO <sub>2</sub> | MgO | Al <sub>2</sub> O <sub>3</sub> | CaO | ZrO <sub>3</sub> | TiO <sub>2</sub> |
|-----------------|--------------------------------|------|------------------|-----|--------------------------------|-----|------------------|------------------|
| 45 Pioneer Mine | 24.60                          | 20.1 | 17.4             | 5.8 | 1.4                            | 2.3 | 2.19             | 1.91             |

Table 6

| Product                        | Wt., percent | Assay, percent                 |      |                  | Distribution, percent          |       |                  | Ratio Cr/Fe |
|--------------------------------|--------------|--------------------------------|------|------------------|--------------------------------|-------|------------------|-------------|
|                                |              | Cr <sub>2</sub> O <sub>3</sub> | Fe   | SiO <sub>2</sub> | Cr <sub>2</sub> O <sub>3</sub> | Fe    | SiO <sub>2</sub> |             |
| Chromite cleaner concentrate 1 | 50.1         | 41.50                          | 23.0 | 1.0              | 84.2                           | 53.3  | 3.1              | 1.23        |
| Chromite cleaner concentrate 2 | 2.9          | 34.26                          | 25.0 | 2.8              | 4.0                            | 3.3   | 0.5              | .94         |
| Chromite cleaner tailing       | 7.6          | 22.40                          | 19.8 | 11.4             | 6.8                            | 7.0   | 5.4              | -----       |
| Rougher tailing                | 39.4         | 3.10                           | 19.9 | 37.3             | 5.0                            | 36.4  | 91.0             | -----       |
| Calculated heads               | 100.0        | 24.7                           | 21.6 | 16.1             | 100.0                          | 100.0 | 100.0            | -----       |

## REAGENTS, POUNDS PER TON OF ORE

|                   | Oleic acid | "Emulsol X-1" | NaF  | H <sub>2</sub> SO <sub>4</sub> | pH    |
|-------------------|------------|---------------|------|--------------------------------|-------|
| Rougher flotation | 0.97       | 0.20          | 2.26 | 3.94                           | 3.1   |
| Cleaner flotation | .25        | 0.05          | 1.97 | .99                            | ----- |

Table 7  
SCREEN ANALYSIS ON PIONEER MINE HIGH CHROMITE SAND

| Product          | Wt., percent | Assay, percent                 |      |                  | Distribution, percent          |       |                  |      |
|------------------|--------------|--------------------------------|------|------------------|--------------------------------|-------|------------------|------|
|                  |              | Cr <sub>2</sub> O <sub>3</sub> | Fe   | SiO <sub>2</sub> | Cr <sub>2</sub> O <sub>3</sub> | Fe    | SiO <sub>2</sub> |      |
| +48-mesh         |              | 5.8                            | 12.3 | 30.5             | 29.7                           | 3.0   | 5.7              | 10.3 |
| -48+65-mesh      |              | 29.8                           | 18.6 | 21.3             | 21.0                           | 23.8  | 30.7             | 38.1 |
| -65+100-mesh     |              | 53.8                           | 24.7 | 20.1             | 14.3                           | 57.6  | 52.5             | 46.9 |
| -100-mesh        |              | 10.6                           | 29.9 | 21.6             | 7.2                            | 15.6  | 11.1             | 4.7  |
| Calculated heads | 100.0        | 22.7                           | 20.7 | 16.4             | 100.0                          | 100.0 | 100.0            |      |

The screen analysis given in the table shows an increase in chromite grade in the finer sizes with silica tending to remain in the coarser sizes. Only a very small amount of minus 200-mesh material was present in the ore.

The procedure for flotation of chromite from the Pioneer mine sands recorded in Table 8 was as follows:

1. Sands as received were pulped with tap water to about 50 percent solids and an emulsion of oleic acid stabilized with "Emulsol X-1" was added until flocculation was pronounced.

5 2. A dilute solution of 10 percent HF was added until the flocs were clean of garnet and gangue.

3. Flotation was carried out until all recoverable chromite had been removed in the froth.

Table 9

## CHROMITE FLOTATION EMPLOYING HYDROGEN FLUORIDE IN PLACE OF FLUORIDE-ACID

| Product                      | Wt., percent | Assay, percent                 |      |                  | Distribution, percent          |       |                  | Ratio Cr/Fe |
|------------------------------|--------------|--------------------------------|------|------------------|--------------------------------|-------|------------------|-------------|
|                              |              | Cr <sub>2</sub> O <sub>3</sub> | Fe   | SiO <sub>2</sub> | Cr <sub>2</sub> O <sub>3</sub> | Fe    | SiO <sub>2</sub> |             |
| Chromite cleaner concentrate | 53.0         | 41.0                           | 20.3 | 2.7              | 79.6                           | 46.8  | 6.6              | 1.38        |
| Chromite cleaner tailing     | 7.2          | 23.6                           | 20.3 | 14.6             | 7.6                            | 7.8   | 6.0              | -----       |
| Rougher tailings             | 49.8         | 5.7                            | 17.0 | 30.8             | 12.8                           | 45.4  | 87.4             | -----       |
| Calculated heads             | 100.0        | 22.2                           | 18.7 | 17.8             | 100.0                          | 100.0 | 100.0            | -----       |

## REAGENTS, POUNDS PER TON OF ORE

|                   | Oleic acid | "Emulsol X-1" | HF   | pH  |
|-------------------|------------|---------------|------|-----|
| Rougher flotation | 1.94       | 0.39          | 0.62 | 3.9 |
| Cleaner flotation |            |               | .50  |     |

1. Sands as received were pulped with tap water to about 50 percent solids, equal amounts of sodium fluoride and sulfuric acid were added and the pulp was conditioned for 2 minutes.

2. An emulsion of oleic acid stabilized with "Emulsol X-1" was added until all the chromite was well flocculated.

3. The pulp was diluted with tap water to about 25 percent solids and all recoverable chromite was floated.

30 The rougher flotation concentrate contained 38.6 percent Cr<sub>2</sub>O<sub>3</sub> and showed a recovery of 87.2 percent of the chromium. By cleaning the rougher flotation concentrate 79.6 percent of the chromium was recovered in a concentrate which assayed 41.0 percent Cr<sub>2</sub>O<sub>3</sub>, 20.3 percent Fe, and 2.7 percent SiO<sub>2</sub>. Results were comparable to those obtained in previous work but the consumption of HF was less in relation to the indi-

Table 8

## CHROMITE FLOTATION EMPLOYING FLUORIDE-ACID TREATMENT AHEAD OF FATTY ACID

| Product                      | Wt., percent | Assay, percent                 |      |                  | Distribution, percent          |       |                  | Ratio Cr/Fe |
|------------------------------|--------------|--------------------------------|------|------------------|--------------------------------|-------|------------------|-------------|
|                              |              | Cr <sub>2</sub> O <sub>3</sub> | Fe   | SiO <sub>2</sub> | Cr <sub>2</sub> O <sub>3</sub> | Fe    | SiO <sub>2</sub> |             |
| Chromite cleaner concentrate | 41.3         | 41.5                           | 20.9 | 1.5              | 77.5                           | 46.4  | 3.6              | 1.36        |
| Chromite cleaner tailing     | 12.7         | 25.2                           | 18.4 | 13.1             | 14.4                           | 12.6  | 9.5              | -----       |
| Rougher tailing              | 46.0         | 3.9                            | 16.6 | 32.0             | 8.1                            | 41.0  | 86.9             | -----       |
| Calculated heads             | 100.0        | 22.1                           | 18.6 | 17.4             | 100.0                          | 100.0 | 100.0            | -----       |

## REAGENTS, POUNDS PER TON OF ORE

|                   | Oleic acid | "Emulsol X-1" | NaF | H <sub>2</sub> SO <sub>4</sub> | pH    |
|-------------------|------------|---------------|-----|--------------------------------|-------|
| Rougher flotation | 4.20       | 0.84          | 2.0 | 2.0                            | 4.4   |
| Cleaner flotation | .25        | .05           | 1.0 | 1.6                            | ----- |

Results show that 91.9 percent of the chromium was recovered in the rougher chromite concentrate at a grade at 38.4 percent Cr<sub>2</sub>O<sub>3</sub>. By 65. cleaning the rougher concentrate, 77.5 percent of the chromium was recovered at 41.5 percent Cr<sub>2</sub>O<sub>3</sub>, 20.9 percent Fe and 1.5 percent SiO<sub>2</sub>. Results were comparable to those obtained in previous work, but the consumption of oleic acid was higher in relation to that of NaF and H<sub>2</sub>SO<sub>4</sub>.

The object of the following test was to study the effect of hydrofluoric acid on the flotation of chromite when it is substituted for the fluoride-sulfuric acid circuit. The procedure employed was as follows:

70 cated consumption in the fluoride-sulfuric acid circuit.

## EXAMPLE V

## LOCKED TESTING

A locked rougher flotation test was run on Pioneer mine sands to determine the effect of returning middlings and flotation water to the circuit. Six rougher tests were run, each of which produced a clean rougher concentrate, a scavenger concentrate, and a rougher tailing. The scavenger concentrate, together with tailing water from each test, was added to the feed in each succeeding test. Combined rougher tailings

were later reground for 5 minutes in a laboratory ball mill and refloated to produce a concentrate and a clean tailing. The combined flotation products were further cleaned by removing magnetite and ilmenite on a disc-type high intensity magnetic separator. The results are given in Tables 10 and 11.

Table 10  
LOCKED TEST ON PIONEER MINE SANDS

| Product                                            | Wt., percent | Assay, percent                 |      |                  | Distribution, percent          |       |                  | Ratio Cr/Fe |
|----------------------------------------------------|--------------|--------------------------------|------|------------------|--------------------------------|-------|------------------|-------------|
|                                                    |              | Cr <sub>2</sub> O <sub>3</sub> | Fe   | SiO <sub>2</sub> | Cr <sub>2</sub> O <sub>3</sub> | Fe    | SiO <sub>2</sub> |             |
| A. Combined rougher chromite concentrate           | 43.8         | 41.4                           | 20.5 | 3.0              | 81.1                           | 48.6  | 7.3              | 1.38        |
| D. Scavenger chromite concet. from No. 8 of series | 7            | 23.0                           | 18.8 | 15.0             | 7                              | 7     | 6                | .84         |
| Combined rougher tailings                          | 55.5         | 7.8                            | 17.0 | 29.4             | 18.2                           | 50.7  | 92.1             | -----       |
| Calculated heads                                   | 100.0        | 22.4                           | 18.4 | 17.8             | 100.0                          | 100.0 | 100.0            | -----       |
| B. Regrind cleaner chromite concentrate            | 5.4          | 36.2                           | 19.2 | 4.8              | 8.7                            | 5.6   | 1.4              | 1.29        |
| C. Regrind cleaner chromite tailings               | 7.0          | 20.9                           | 16.3 | 17.0             | 6.5                            | 6.1   | 6.7              | .88         |
| Regrind rougher tailings                           | 43.1         | 1.5                            | 16.8 | 34.6             | 3.0                            | 39.0  | 84.0             | -----       |
| Calculated rougher tailings                        | 55.5         | 7.3                            | 17.0 | 29.4             | 18.2                           | 50.7  | 92.1             | -----       |

## TOTAL REAGENTS, POUNDS PER TON OF ORE

|                           | Oleic acid | "Emulsol X-1" | NaF  | H <sub>2</sub> SO <sub>4</sub> | Average pH |
|---------------------------|------------|---------------|------|--------------------------------|------------|
| Rougher flotation         | 2.38       | 0.48          | 0.59 | 1.60                           | 3.5        |
| Regrind rougher flotation | .66        | .14           | .54  | 1.32                           | 3.3        |
| Regrind cleaner flotation | .20        | .04           | .13  | .33                            | 3.4        |

The results of the locked flotation tests indicated that the middlings would not build up in a continuously operated flotation circuit and that recovery and grade of concentrate are not lowered by return of middlings to the flotation circuit. A chromite concentrate was made assay-ing 41.4 percent Cr<sub>2</sub>O<sub>3</sub> and containing 81.1 percent of the chromite in the ore. The regrinding and reflootation of the rougher flotation tailing indicated that a large part of the chromite lost in the rougher tailing could be recovered in a medium-grade product.

35 aqueous pulp of such an ore in the presence of hydrofluoric acid, and a long-chain fatty acid at a pulp acidity of between pH 1.5 and pH 5.5, and separating a chromium-containing froth as a concentrate.

40 2. In a process for the beneficiation of chromium ores the steps which comprise agitating and aerating aqueous pulp of a comminuted chromite ore in the presence of a long-chain fatty acid, and an acidic fluorine compound at a pulp acidity between pH 2.5 and pH 4.5, and recovering a 45 froth containing a chromite concentrate.

Table 11  
MAGNETIC SEPARATION OF FLOTATION CONCENTRATES [OBTAINED FROM LOCKED TEST

| Product                              | Wt., percent | Assay, percent                 |      |                  | Distribution, percent          |      |                  | Ratio Cr/Fe |
|--------------------------------------|--------------|--------------------------------|------|------------------|--------------------------------|------|------------------|-------------|
|                                      |              | Cr <sub>2</sub> O <sub>3</sub> | Fe   | SiO <sub>2</sub> | Cr <sub>2</sub> O <sub>3</sub> | Fe   | SiO <sub>2</sub> |             |
| Nonmagnetic from product A           | 38.8         | 45.3                           | 18.9 | 2.0              | 77.1                           | 39.6 | 0.3              | 1.64        |
| Magnetic from product A              | 5.0          | 18.2                           | 33.4 | 0.8              | 4.0                            | 9.0  | 7.0              | -----       |
| Calculated heads product A           | 43.8         | 42.2                           | 20.6 | 1.9              | 81.1                           | 48.6 | 7.3              | -----       |
| Nonmagnetic from products A and B    | 43.1         | 44.5                           | 18.4 | 2.4              | 84.7                           | 43.2 | 0.8              | 1.65        |
| Magnetic from products A and B       | 6.1          | 18.8                           | 33.0 | 1.6              | 5.1                            | 11.0 | 7.9              | -----       |
| Calculated head products A and B     | 49.2         | 41.3                           | 20.2 | 2.3              | 89.8                           | 54.2 | 8.7              | -----       |
| Nonmagnetic from products A, B, C, D | 50.0         | 41.9                           | 18.0 | 4.4              | 91.4                           | 49.0 | 0.8              | 1.59        |
| Magnetic from products A, B, C, D    | 6.9          | 19.0                           | 32.2 | 1.6              | 5.6                            | 12.0 | 15.2             | -----       |
| Calculated head products A, B, C, D  | 56.9         | 39.1                           | 19.7 | 4.1              | 97.0                           | 61.0 | 18.0             | -----       |

The use of magnetic separation to remove small amounts of magnetite and ilmenite from flotation concentrates would permit plus 90 percent recoveries at 41.9 percent Cr<sub>2</sub>O<sub>3</sub> grade or grades up to 45.0 percent Cr<sub>2</sub>O<sub>3</sub> with lower recoveries.

As shown in the foregoing examples, the flotation procedure can be followed by a magnetic concentration further to remove magnetic iron compounds from the concentrate secured by flotation to yield a still higher grade concentrate.

3. In a process for the beneficiation of chromium ores, the improvement which comprises agitating and aerating an aqueous pulp of a comminuted chromite ore in the presence of a long-chain fatty acid, a dispersing agent, and a soluble fluoride at a pulp acidity between pH 1.5 and pH 5.5, and recovering a froth containing a chromite concentrate.

4. In a process for the beneficiation of chromium ores, the improvement which comprises agitating and aerating a chromite ore pulp comminuted to a particle size between minus 20-

13

mesh and minus 800-mesh in the presence of, per ton of ore, from 0.1 to 10 pounds of a soluble fluoride, from 0.5 to 5 pounds of a long-chain fatty acid having from 8 to 18 carbon atoms, and an amount of a strong mineral acid sufficient to maintain the pulp acidity between pH 2.5 and pH 4.5, and recovering a chromite concentrate as a floated product.

5. In a process for the beneficiation of chromium ores, the improvement which comprises 10

14

agitating and aerating an aqueous pulp of a chromite ore comminuted to a particle size between minus 48-mesh and minus 200-mesh in the presence of, per ton of ore, from 0.6 to 7.0 pounds of sodium fluoride, from 1 to 4.5 pounds of oleic acid and from 1 to 11 pounds of sulfuric acid, and recovering a chromite concentrate as a floated product.

RICHARD HAVENS.